

E. C. Thayer

Machine Belting.

No 26,151.

Patented Dec. 13, 1859.



Witnesses:  
Joseph S. Pitman  
Henry Hale

Inventor:  
E. C. Thayer

# UNITED STATES PATENT OFFICE.

EUCLID C. THAYER, OF PROVIDENCE, RHODE ISLAND.

## BELTING FOR PULLEYS.

Specification of Letters Patent No. 26,451, dated December 13, 1859.

*To all whom it may concern:*

Be it known that I, EUCLID C. THAYER, of the city and county of Providence, in the State of Rhode Island and Providence Plantations, have invented a new and useful manufacture, to wit: an Improved Round Belting for Grooved Pulleys, which is fully described in the following specification, reference being had to the accompanying drawings.

A strip of leather or other material of which the belting is to be made, is prepared as represented in Fig. 1 by A, B, C, D, of such width and thickness as may be required, by shaving the edges or in any other mode so that its transverse section as seen at A, s, t, B, is in an elliptical form or nearly so; the more perfect the ellipse the greater the perfection of the belting. The material being so prepared, the belt is made by rolling and twisting the material in the following manner: Commencing at the corner A the leather or other material is rolled from that corner to the points a, b, c, or d, according as a greater or less number of overlapping layers is required to make the belt of the requisite size and strength, forming at the ends A, B, a cylinder F, and as the process of rolling is continued the material is twisted so that the strip is rolled up spirally, the same inclination of the spiral fold being preserved to the end of the belt. A belt constructed in this manner may be made of any length by lapping and cementing additional strips at the end C, D, either at right angles with the length of the strip or diagonally. As the rolling and twisting proceeds a cement is placed upon the surfaces of the strip by which the overlying folds are firmly secured together and the more firmly than if the material was rolled in any other way.

I prefer to so roll the material as to leave a cylindrical space in the center of the belt by means of which greater flexibility is se-

cured to it, but the belt may be so made that when finished it will be solid. When the belt is made of leather this spiral rolling and twisting greatly increases the strength of the belt for the fibers of the leather are crossed in every direction, and furthermore if the leather is weak in any part the weak points of the leather will be overlapped by the stronger portions and thus a more uniform strength obtained.

When the belt is in use if the strain upon it should cause the fibers of the belt to give way at the overlapping edge as at h, the break being generally in a direction at right angles with the spiral fold, would soon be arrested by the strength of the under portions of the belt and by the overlapping edge. The spiral form of the belt as above made prevents the edges of the leather opening by the giving way of the cement, and when, combined with a cylindrical space in the center of the belt imparts greater flexibility and elasticity, at the same time securing greater strength and durability than any other form while the tension of the belt on the pulleys keeps the twist in the belt firm and taut.

I do not claim rolling leather or other material into round belting for machinery and cementing the overlapping surfaces.

I claim—

The manufacture of round belting by preparing the leather or other material in the mode described and rolling and twisting the same in a spiral form with any required number of conical layers in the cylinder either with or without a cylindrical space in the center of the belt and cementing the layers in the process of manufacture substantially as described.

EUCLID C. THAYER.

Witnesses:

JOSEPH T. PITMAN,  
HENRY EARLE.